

# United States Patent Office

3,081,170  
Patented Mar. 12, 1963

1

3,081,170

## FOG REDUCTION IN PHOTOGRAPHIC SILVER HALIDE EMULSIONS

Emil B. Rauch and Fritz Dersch, Binghamton, N.Y., assignors to General Aniline & Film Corporation, New York, N.Y., a corporation of Delaware  
No Drawing. Filed Oct. 6, 1958, Ser. No. 765,339  
16 Claims. (Cl. 96—109)

This invention relates to photographic materials and to methods of preparing them. More particularly, this invention relates to light-sensitive silver halide emulsions containing as a stabilizing and antifogging agent an N-substituted-3-aminomethylazolethione. 10

It is well known in the photographic art that light-sensitive emulsions, such as gelatino-silver halide emulsions, have a tendency to fog. Fog is usually caused by a prolonged ripening of the emulsion, by prolonged storage especially at elevated temperatures and humidity, and by prolonged development. To overcome this undesirable property, it has been the practice in this art to add certain chemical compounds to the emulsions to increase their stability and to reduce their tendency to fog. However, the stabilizing and antifogging compounds heretofore used in this art have the disadvantage that upon addition to the emulsion they cause a loss of speed and/or contrast of the emulsion. 15

It is, accordingly, an object of this invention to produce a light-sensitive emulsion which is fast, stable, has a reduced tendency to fog and has good contrast. 20

A further object of this invention resides in a light-sensitive emulsion which contains a compound which stabilizes the emulsion against fogging and at the same time does not materially reduce the speed and/or the contrast of the emulsion. 25

We have discovered that N-substituted-3-aminomethylazolethiones when added to a light-sensitive silver halide emulsion, stabilize and inhibit the fogging of the emulsion. 30

The azolethiones, the use of which is contemplated herein, may be represented by the following formulae: 35



and



wherein R and R<sub>1</sub> are hydrogen atoms or alkyl radicals, e.g., methyl, ethyl, propyl, isopropyl, butyl, isobutyl, amyl, dodecyl and the like; and acyl radical, e.g., acetyl, propionyl and the like; a carboxyalkoxy radical, e.g., carboxymethoxy, carboxyethoxy, carboxypropoxy, X represents alkyl, e.g., methyl, ethyl, propyl, isopropyl, butyl, isobutyl, amyl, isoamyl, chloroethyl, carboxymethyl, allyl; aryl, e.g., phenyl, naphthyl, tetrahydronaphthyl, aralkyl, e.g., benzyl, phenethyl; X' represents hydrogen or a substituent having the value stated for X; and wherein X and X' together represent the atoms necessary to complete a heterocyclic, hydrogenated ring system, e.g., a piperidine, tetrahydroquinoline, morpholine or 60

65  
70

2

piperazine ring system, Y is an oxygen, selenium or sulfur atom, and Z represents the atoms necessary to complete a fused-on aromatic ring system such as a benzo or naphtho ring which can be further substituted. 5

The following specific compounds are examples of compounds belonging to the class of compounds having the general formula given above which we have found suitable for use as stabilizing an antifogging agents: 10



3-piperidinomethyl-benzoxazole-2-thione



1,4-bisbenzoxazole-2-thione-3-methylpiperazine



3-morpholinomethylbenzoxazole-2-thione



3-diethylaminomethyl-benzoxazole-2-thione



3-dibutylaminomethyl-benzoxazole-2-thione



3-piperidinomethyl-benzothiazole-2-thione



3-morpholinomethyl-benzothiazole-2-thione



These compounds are prepared by reacting a 2-mercapto-substituted azole of the oxazole, benzoxazole, selenazole, benzoselenazole, thiazole and benzothiazole series simultaneously with formaldehyde and a primary or secondary amine in the presence of a suitable solvent such as methanol, ethanol, isopropanol and the like. The preparation of these compounds is described in more detail in U.S. Patent 2,411,253, British patent 377,253; and Journal of the Chemical Society, 1948, page 1717.

As representatives of azoles used in the reaction the following are mentioned:

- 4-methyl-2-mercaptopthiazole
- 4-ethyl-2-mercaptopthiazole
- 4-propyl-2-mercaptopthiazole
- 4-dodecyl-2-mercaptopthiazole
- 4-butyl-2-mercaptopthiazole
- 4-phenyl-2-mercaptopthiazole
- 4-p-chlorophenyl-2-mercaptopthiazole
- 4-p-methoxyphenyl-2-mercaptopthiazole
- 4,5-propano-2-mercaptopthiazole
- 4,5-dimethyl-2-mercaptopthiazole
- 4,5-diphenyl-2-mercaptopthiazole
- 4,5-diethyl-2-mercaptopthiazole
- 5-carbomethoxy-4-methyl-2-mercaptopthiazole
- 5-methyl-2-mercaptopbenzothiazole
- 6-methyl-2-mercaptopbenzothiazole
- 7-methyl-2-mercaptopbenzothiazole
- 6-tert-butyl-2-mercaptopbenzothiazole
- 6-phenyl-2-mercaptopbenzothiazole
- 5-hydroxy-2-mercaptopbenzothiazole
- 5-chloro-2-mercaptopbenzothiazole
- 5-bromo-2-mercaptopbenzothiazole
- 6-chloro-2-mercaptopbenzothiazole
- 6-bromo-2-mercaptopbenzothiazole
- 6-nitro-2-mercaptopbenzothiazole
- 5-amino-2-mercaptopbenzothiazole
- 6-amino-2-mercaptopbenzothiazole
- 6-acetamido-2-mercaptopbenzothiazole
- 6-benzamido-2-mercaptopbenzothiazole
- 6-dimethylamino-2-mercaptopbenzothiazole
- 5-carboxyl-2-mercaptopbenzothiazole
- 4,6-dimethyl-2-mercaptopbenzothiazole
- 4-methyl-6-chloro-2-mercaptopbenzothiazole
- 5,6-dichloro-2-mercaptopbenzothiazole
- 4-carboxy-6-chloro-2-mercaptopbenzothiazole
- 4,6-dimethyl-7-chloro-2-mercaptopbenzothiazole
- 4,6-dimethyl-5,7-dichloro-3-mercaptopbenzothiazole
- 4,5-benzo-2-mercaptopbenzothiazole
- 6,7-benzo-2-mercaptopbenzothiazole
- 2-mercaptop-4,5,6,7-dibenzothiazole
- 2-mercaptop-5,6-naphthobenzothiazole
- 2-mercaptop-5,6-benzothiazole
- 2-mercaptop-4,5-fluorenyl (1,2)-thiazole
- 6,7-benzo-2-mercaptopbenzoselenazole
- 2-mercaptopbenzoselenazole
- 2-mercaptoselenazole

- 2-mercaptop-5-methoxybenzoselenazole
- 2-mercaptop-5-methylbenzoselenazole
- 2-mercaptop-6-methoxyquinoline
- 2-mercaptop-6-methylquinoline
- 2-mercaptopbenzoxazole
- 2-mercaptop-5-phenylbenzoxazole
- 2-mercaptop-5-methoxybenzoxazole
- 2-mercaptop-5-methylbenzoxazole
- 2-mercaptop-4,5-benzobenzoxazole
- 10 The following list is representative of primary and secondary amines, the latter including cyclic amines, which can be condensed with formaldehyde and the mercaptoazoles:
- 15 Methylamine
- Ethylamine
- $\beta$ -Hydroxyethylamine
- $\beta$ -Chloroethylamine
- Allylamine
- 20 Benzylamine
- $\beta$ -Phenylethylamine
- Ethylenediamine
- Ethyl aminoacetate
- $\omega$ -Aminoacetophenone
- 25 Tetrahydro- $\beta$ -naphthylamine
- Aniline
- 3,4-methylene-dioxybenzylamine
- Dimethylamine
- Diethylamine
- 30 Diethanolamine
- Dipropylamine
- Di-n-butylamine
- Diisoamylamine
- Dibenzylamine
- 35 methyl-diethylethylenediamine
- Methylaniline
- Piperidine
- 1,2,3,4-tetrahydroisoquinoline
- 6-methoxy-1,2,3,4-tetrahydroisoquinoline
- 40 Morpholine
- Piperazine
- $\omega$ -Methylaminopropiophenone
- $\beta$ -Acetylethylbenzylamine
- Benzyl-(2-cyclohexanonylmethyl)-amine
- 45 3,4-methylenedioxybenzyl-(2-cyclohexanonylmethyl)-amine
- The antifogging agents of our invention may be added to the emulsion at any stage during its process of production. Thus, they may be added as a "ripening final" or as a "coating final." When added as a "ripening final," they are added during the ripening or sensitivity increasing stage of the emulsion making process. Such addition may be made before, during or after the addition of the soluble silver salt to the soluble halide in the presence of a suitable colloid, such as gelatin, polyvinyl alcohol, solubilized casein or albumin. When added as a "coating final," the antifogging agent of our invention is added to the emulsion just prior to coating it on a suitable support such as glass, paper, or film at a time when the emulsion has nearly attained its maximum sensitivity.
- 50 In some instances, it is advantageous to apply the antifogging and stabilizing compounds of our invention in a separate layer such as an undercoating layer or in an anti-abrasion gelatin surface. Sometimes it is desirable to incorporate the compounds in one or all processing baths
- 55 or in the pre- and post-baths.
- When used as a "ripening final," the antifogging agents of our invention are preferably added to the emulsion in an amount ranging from 0.1 milligram to 20 milligrams per 0.6 mol of silver halide and when used as a "coating final," it is preferably added in an amount ranging from 0.5 milligram to 50 milligrams per 0.6 mol of silver halide. The optimum amount to be added depends primarily on the type of emulsion and should be determined individually in each case.
- 70 75 The stabilizers and antifogging agents of our invention may



wherein R and R<sub>1</sub> are selected from the group consisting of hydrogen, alkyl, acyl and carboxyalkoxy; Z represents the atoms necessary to complete a fused-on aromatic ring structure of the benzene and naphthalene series; Y is a member selected from the group consisting of oxygen and sulfur; A is a member selected from the class consisting of



10

and



15

wherein X and X<sub>1</sub> are selected from the group consisting of hydrogen, alkyl, aryl and aralkyl, X<sub>1</sub> being a substituent other than hydrogen when X is hydrogen, and X<sub>2</sub> represents the atoms necessary to complete a hydrogenated heterocyclic ring system of the piperidine and morpholine series.

2. A light-sensitive photographic element comprising a base and a coating of gelatino-silver halide emulsion thereon, said emulsion containing as an antifogging and stabilizing agent, a compound selected from the group having the following formulae:



20

and



25

and



30

wherein R and R<sub>1</sub> are selected from the group consisting of hydrogen, an aliphatic radical, an aromatic radical; Z represents the atoms necessary to complete a fused-on aromatic ring structure, Y is a member selected from the group consisting of oxygen and sulfur, A is a member selected from the class consisting of



40

and



45

wherein X and X<sub>1</sub> are selected from the group consisting of hydrogen, aliphatic, aryl and aralkyl radicals, X<sub>1</sub> being a substituent other than hydrogen when X is hydrogen, and wherein X<sub>2</sub> represents the atoms necessary to complete a hydrogenated heterocyclic ring system of the piperidine and morpholine series.

3. A light-sensitive structure comprising a base, a

layer of light-sensitive silver halide emulsion thereon, and a separate layer adjacent said first mentioned layer containing as an antifogging and stabilizing agent compound, a compound selected from the group having the following general chemical structures:



and



and



wherein R and R<sub>1</sub> are selected from the group consisting of hydrogen, an aliphatic radical, an aromatic radical; Z represents the atoms necessary to complete a fused-on aromatic ring structure, Y is a member selected from the group consisting of oxygen and sulfur, A is a member selected from the class consisting of



and



wherein X and X<sub>1</sub> are selected from the group consisting of hydrogen, aliphatic, aryl and aralkyl radicals, X<sub>1</sub> being a substituent other than hydrogen when X is hydrogen, wherein X<sub>2</sub> represents the atoms necessary to complete a hydrogenated heterocyclic ring system of the piperidine and morpholine series.

4. A process of forming a photographic silver halide emulsion having a reduced tendency to fog which comprises forming the emulsion, ripening the emulsion and during said ripening adding thereto a compound selected from the group having the following general formulae:



and



70

75

and



wherein R and R<sub>1</sub> are selected from the group consisting of hydrogen, an aliphatic radical, an aromatic radical; Z represents the atoms necessary to complete a fused-on aromatic ring structure, Y is a member selected from the group consisting of oxygen and sulfur, A is a member selected from the class consisting of



and



wherein X and X<sub>1</sub> are selected from the group consisting of hydrogen, aliphatic, aryl and aralkyl radicals, X<sub>1</sub> being a substituent other than hydrogen when X is hydrogen, and wherein X<sub>2</sub> represents the atoms necessary to complete a hydrogenated heterocyclic ring system of the piperidine and morpholine series.

5. A process of forming a light-sensitive photographic element having a reduced tendency to fog which comprises forming a silver halide emulsion, ripening said emulsion, coating said emulsion on a base and adding to said emulsion just prior to the coating thereof on the base a compound selected from the group having the following general formulae:



and



and



wherein R and R<sub>1</sub> are selected from the group consisting

of hydrogen, alkyl, acyl and carboxyalkoxy; Z represents the atoms necessary to complete a fused-on aromatic ring structure of the benzene and naphthalene series; Y is a member selected from the group consisting of oxygen and sulfur; A is a member selected from the class consisting of



and



15 wherein X and X<sub>1</sub> are selected from the group consisting of hydrogen, alkyl, aryl and aralkyl, X<sub>1</sub> being a substituent other than hydrogen when X is hydrogen, and X<sub>2</sub> represents the atoms necessary to complete a hydrogenated heterocyclic ring system of the piperidine and morpholine series.

6. A light-sensitive silver halide emulsion as recited in claim 1, wherein the antifogging and stabilizing compound is 3-morpholinomethyl-benzothiazole-2-thione.

25 7. A light-sensitive silver halide emulsion as recited in claim 1, wherein the antifogging and stabilizing compound is 3-piperidinomethyl-benzoxazole-2-thione.

8. A light-sensitive halide emulsion as recited in claim 1, wherein the antifogging and stabilizing compound is 3-dimethylaminomethyl-benzoxazole-2-thione.

20 9. A light-sensitive silver halide emulsion as recited in claim 1, wherein the antifogging and stabilizing compound is 3-morpholinomethylbenzoxazole-2-thione.

10. A light-sensitive silver halide emulsion as recited 35 in claim 1, wherein the antifogging and stabilizing compound is 3-diethylaminomethyl-benzoxazole-2-thione.

11. A light-sensitive silver halide emulsion as recited in claim 1, wherein the antifogging and stabilizing compound is 3-piperidinomethyl-benzothiazole-2-thione.

40 12. A light-sensitive silver halide emulsion as recited in claim 1, wherein the antifogging and stabilizing compound is present in the emulsion in the ratio of 0.1 to 50 milligrams per 0.6 mol of silver halide.

13. A light-sensitive silver halide emulsion as recited 45 in claim 1, wherein the antifogging and stabilizing compound is present in the emulsion in the ratio of 0.1 to 20 milligrams per 0.6 mol of silver halide.

14. A light-sensitive silver halide emulsion as recited 50 in claim 1, wherein the antifogging and stabilizing compound is present in the emulsion in the ratio of 0.5 to 50 milligrams per 0.6 mol of silver halide.

15. A light-sensitive silver halide emulsion as recited in claim 1, wherein said emulsion is a panchromatic emulsion.

55 16. A light-sensitive silver halide emulsion as recited in claim 1, containing the reaction product of a long chain alcohol and ethylene oxide as an accelerator.

#### References Cited in the file of this patent

#### UNITED STATES PATENTS

- |           |               |       |               |
|-----------|---------------|-------|---------------|
| 2,099,374 | Schwarz       | ----- | Nov. 16, 1937 |
| 2,453,346 | Russell       | ----- | Nov. 9, 1948  |
| 2,819,965 | Murray et al. | ----- | Jan. 14, 1958 |
| 2,870,015 | Allen et al.  | ----- | Jan. 20, 1959 |

UNITED STATES PATENT OFFICE  
CERTIFICATE OF CORRECTION

Patent No. 3,081,170

March 12, 1963

Emil B. Rauch et al.

It is hereby certified that error appears in the above numbered patent requiring correction and that the said Letters Patent should read as corrected below.

Column 7, lines 55 and 56, column 8, lines 34 and 35, and column 9, lines 12 and 13, for "an aliphatic radical, an aromatic radical;", each occurrence, read -- alkyl, acyl and carboxyalkoxy; --; column 7, line 57, column 8, line 36, and column 9, line 14, for "structure,", each occurrence, read -- structure of the benzene and naphthalene series; --; column 7, line 58, column 8, line 37, and column 9, line 15, for "sulfur,", each occurrence, read -- sulfur; --; column 7, line 70, column 8, line 49, and column 9, line 26, for "aliphatic, aryl and aralkyl radicals,", each occurrence, read -- alkyl, aryl and aralkyl, --; column 7, line 72 and column 9, line 29, strike out "wherein", each occurrence; column 8, line 51, for "wherein" read -- and --.

Signed and sealed this 24th day of November 1964.

(SEAL)  
Attest:

ERNEST W. SWIDER  
Attesting Officer

EDWARD J. BRENNER  
Commissioner of Patents